

## UNITED STATES PATENT OFFICE

2,685,515

## PHOTOGRAPHIC DEVELOPER COMPOSITION

Charles V. Wilson, Rochester, N. Y., assignor to  
Eastman Kodak Company, Rochester, N. Y., a  
corporation of New Jersey

No Drawing. Application August 3, 1953,  
Serial No. 372,191

15 Claims. (Cl. 95—88)

1

This invention relates to photographic developers and particularly to methods for accelerating the development rate of photographic developing agents.

A class of silver halide developing agents has come under consideration which in themselves are very weak developing agents for silver halide emulsions even under the most favorable conditions for development. Examples of such compounds are as follows:



2

These ene-diol compounds, except for dihydro-pyrogallol, have the following general formula



5 10 wherein R represents a substituent such as an alkyl group preferably containing from 1 to 4 carbon atoms e. g. methyl, ethyl, n-propyl and n-butyl, an alkoxy group e. g. methoxy, or a halogen atom e. g. chlorine and bromine, and Z represents 15 either a sulfur or oxygen atom, or a methylene group, imino group or the N-alkyl group =NR<sub>1</sub> in which R<sub>1</sub> preferably contains from 1 to 4 carbon atoms e. g. a N-methyl, N-ethyl, N-n-propyl or N-n-butyl group. The equilibrium forms of 20 these compounds, such as those shown hereinabove, are contemplated in the developers of our invention.

It is considered that the active portion of the molecule is that containing the cyclic ene-diol system. The compounds are not to be confused with polyhydric aromatic compounds such as catechol or pyrogallol which show serious disadvantages such as a strong tendency to form colored oxidation products in the development reaction or on contact with the oxygen in the air, which products discolor solutions and stain photographic materials.

We have discovered that the developing rate of developing solutions containing the above 35 ene-diol compounds can be markedly accelerated by the addition to developing solutions containing the ene-diol compounds, of 3-pyrazolidone compounds which themselves are only moderately active developing agents for silver halide. 40 The activity of the resulting developer solution containing both the ene-diol and pyrazolidone compounds is very much greater than would be expected from summing up the separate activities. An added feature of the ene-diol-pyrazolidone developer compositions resides in the stability of the developing solution; that is, 3-pyrazolidone compounds such as 1-phenyl-3-pyrazolidone are highly unstable in alkaline developer compositions free of a preservative and tend to 50 darken and lose development activity quickly particularly through aerial oxidation. On the other hand, when development is carried out with the 3-pyrazolidone compounds in the presence of the ene-diol compounds, the latter function as preservatives and the developer is highly resistant to discoloration and loss of activity. Another advantageous characteristic of the ene-diol-pyrazolidone developer compositions is that the developers show little tendency for the formation 55 of silver sludge or for the formation of dichroic 60

stain on silver images. A further characteristic of the ene-diol-pyrazolidone developer compositions of the invention resides in the fact that the compositions behave as strong surface latent image developers as opposed to internal latent image developers, as long as they are free of silver halide solvents such as sodium sulfite. That is, developer compositions containing 3-pyrazolidone compounds have been described in the literature but invariably they have been compounded so as to contain a silver halide solvent such as sodium sulfite as a preservative. In order to convert such a developer composition to a surface latent image developer we have found it to be necessary to dispense with the silver halide solvent in the developer composition. However, as mentioned, the 3-pyrazolidone developers free of preservative are very unstable. When, according to our invention, the ene-diol compounds are incorporated into the 3-pyrazolidone developer compositions, the ene-diol compounds supply the required preservative effect and the surface latent image developer characteristics are maintained. Therefore, the fortuitous choice of 3-pyrazolidone compounds to accelerate the development rate of the ene-diol compounds has resulted in the latter compounds exerting a complementary preservative effect as well as providing a stable 3-pyrazolidone developer system which has surface latent image development characteristics and shows no tendency for physical development. For these reasons the developers of the invention are very useful in color development processes where a black and white developer is required.

An additional unexpected feature of the developers containing the 3-pyrazolidone and ene-diol compounds resides in the fact that similar developer compositions can be prepared in which the pyrazolidone is replaced by a conventional developing agent, for example, containing a mixture of N-methyl-p-aminophenol and dihydropyrogallol, which compositions do not exhibit the mentioned development acceleration effect to anything like the same degree.

The 3-pyrazolidone developer compositions of the invention containing the above ene-diol compounds can be readily converted to internal latent image developer compositions by merely adding a silver halide solvent such as sodium thiosulfate thereto. The resultant internal latent image developer composition, by virtue of the presence of one of the mentioned ene-diol compounds, possesses satisfactory keeping properties even in the absence of the usual sulfite preservative.

The 3-pyrazolidone silver halide developing agents employed in the developer compositions together with the ene-diols, have the general structure



in which the R groups each represent various substituents such as hydrogen, alkyl or aryl groups, for example R<sub>1</sub> can be hydrogen or a group such as alkyl preferably containing from 1 to 4 carbon atoms, or an aryl group of the benzene or naphthalene series substituted or not, and R<sub>2</sub>, R<sub>3</sub>, R<sub>4</sub> and R<sub>5</sub> can be hydrogen atoms or alkyl as above or aryl such as phenyl.

The following compounds are representative of 3-pyrazolidone silver halide developing agents

which are useful in the developer compositions of the invention:

1. 1-phenyl-3-pyrazolidone
2. 1-p-tolyl-3-pyrazolidone
3. 5-phenyl-3-pyrazolidone
4. 5-methyl-3-pyrazolidone
5. 1-p-chlorophenyl-3-pyrazolidone
6. 1-phenyl-5-phenyl-3-pyrazolidone
7. 1-m-tolyl-3-pyrazolidone
8. 1-phenyl-5-methyl-3-pyrazolidone
9. 1-p-tolyl-5-phenyl-3-pyrazolidone
10. 1-m-tolyl-3-pyrazolidone
11. 1-p-methoxyphenyl-3-pyrazolidone
12. 1-acetamidophenyl-3-pyrazolidone
13. 1-phenyl-2-acetyl - 4,4 - dimethyl - 3 - pyrazolidone
14. 1-phenyl-4,4-dimethyl-3-pyrazolidone
15. 1-m-aminophenyl - 4 - methyl - 4 - propyl-3-pyrazolidone
16. 1-o-chlorophenyl - 4 - methyl - 4 - ethyl - 3-pyrazolidone
17. 1 - m - acetamidophenyl - 4,4 - diethyl - 3-pyrazolidone
18. 1 - (p -  $\beta$  - hydroxyethylphenyl) - 4,4 - dimethyl-3-pyrazolidone
19. 1 - p - hydroxyphenyl - 4,4 - dimethyl - 3-pyrazolidone
20. 1 - p - methoxyphenyl - 4,4 - diethyl - 3-pyrazolidone
21. 1-p-tolyl-4,4-dimethyl-3-pyrazolidone
22. 1 - (7 - hydroxy - 2 - naphthyl) - 4 - methyl-4-n-propyl-3-pyrazolidone
23. 1-p-diphenyl-4,4-dimethyl-3-pyrazolidone
24. 1-(p- $\beta$ -hydroxyethylphenyl)-3-pyrazolidone
25. 1-o-tolyl-3-pyrazolidone
26. 1-o-tolyl-4,4-dimethyl-3-pyrazolidone

The 4,4-dialkyl-3-pyrazolidone compounds 13 to 23 and 26 above are particularly efficacious for use in the developer compositions of our invention inasmuch as they are more active developing agents than are compounds 1 to 12 which contain a single substituent or only hydrogen atoms in the 4-position of the pyrazolidone nucleus. The 4,4-dialkyl-3-pyrazolidone compounds are described and claimed in the Allen et al. U. S. patent application Serial No. 372,148 filed concurrently herewith. The  $\omega$ -hydroxy-alkylphenyl-3-pyrazolidones, for example, compounds 18 and 24 above, are also especially useful in concentrated formulas, in replenishers and in the presence of high salt concentrations where their increased solubility enables obtaining and holding adequate amounts of the pyrazolidone compound in solution. The compounds are described and claimed in the Allen et al. U. S. patent application Serial No. 372,148 filed concurrently herewith and in the Reynolds and Tinker U. S. patent application Serial No. 372,167 filed concurrently.

#### Example 1

A developer of the following composition was prepared:

|                             | Grams |
|-----------------------------|-------|
| 65 1-phenyl-3-pyrazolidone  | 0.4   |
| Dihydropyrogallol           | 2.56  |
| Sodium sulfite              | 25    |
| Sodium sesquicarbonate      | 22.6  |
| Sodium hydroxide to pH 10.0 |       |
| 70 Water to 1 liter.        |       |

The solution was used to develop a fine-grain positive film, a density of 0.95 being obtained after 2 minutes' development. The same solution containing only dihydropyrogallol as the developing

agent required 32 minutes to develop a density of 0.31 and when the solution contained only 1-phenyl-3-pyrazolidone as the developing agent, the film developed to a density of only 0.30 in 2 minutes.

*Example 2*

The following developer composition is suitable for use as a negative developer for color films:

|                               | Grams/liter |
|-------------------------------|-------------|
| Sodium hexametaphosphate      | 0.5         |
| Sodium sulfite                | 40.0        |
| Sodium carbonate monohydrate  | 25.0        |
| Potassium bromide             | 1.0         |
| Potassium iodide              | 0.002       |
| 1-Phenyl-3-pyrazolidone       | 1.0         |
| Dihydropyrogallol             | 7.1         |
| 1-Phenyl-5-marcapto tetrazole | 0.01        |
| Water to make 1.0 liter.      |             |

The developer of this example can be used in any of the well-known processes of color development where a black-and-white developer is required. The developer is especially useful in mixed grain color processes employing films such as disclosed in Mannes et al. U. S. Patent 2,388,856 or in the Carroll et al. U. S. Patent 2,614,925, October 21, 1952, wherein, for example, is shown a two-layer film, one layer containing blue-sensitive silver halide, the other containing a mixture of green and red-sensitive silver halide grains. When the developer immediately above is used, particularly if the formula is free of sulfite, in the color process of the patents as the negative developer for such a film it is observed that physical development effects are minimized with the result that the color developed images have increased saturation because of decreased physical development in the negative developer of the invention.

Results similar to those shown in the above examples are obtained when the developer compositions either containing or free of silver halide solvents are prepared from mixtures of at least one of the indicated 3-pyrazolidone compounds and at least one of the indicated ene-diol compounds. Particularly valuable developer compositions in addition to that exemplified above are those containing dihydropyrogallol and either a 1-tolyl-3-pyrazolidone such as 1-p-tolyl-3-pyrazolidone or 1-p-tolyl-4,4-dimethyl-3-pyrazolidone or a 1-(p-hydroxyalkylphenyl)-4,4-dialkyl-3-pyrazolidone such as 1-(p- $\beta$ -hydroethylphenyl)-4,4-dimethyl-3-pyrazolidone, or a 1-(p-hydroxyalkylphenyl)-3-pyrazolidone such as 1-(p- $\beta$ -hydroxyethylphenyl)-3-pyrazolidone.

It will be understood that our invention, as specified by the claims hereinafter, includes the mentioned developer compositions in either the liquid form exemplified above, or in the dry powder form such as packaged developer formulas suitable for dissolving in water to form a liquid developer. Such dry compositions include the mentioned 3-pyrazolidone compounds, the ene-diol compound, and alkaline material such as sodium carbonate, caustic alkali or sodium perborate.

What I claim is:

1. A photographic developer composition comprising an alkaline material, a 3-pyrazolidone silver halide developing agent and a member of

the group consisting of compounds having the general formula



wherein R represents a member of the group consisting of an alkyl group of from 1 to 4 carbon atoms, an alkoxy group of from 1 to 4 carbon atoms and a halogen atom, and Z represents a member of the group consisting of an N-alkyl group of from 1 to 4 carbon atoms, a methylene group, an imino group, a sulfur atom and an oxygen atom, and dihydropyrogallol.

2. A photographic developer composition comprising an aqueous alkaline solution containing a mixture of a 3-pyrazolidone silver halide developing agent and a compound selected from the group consisting of a coumarindiol; a thiacoumarindiol; a carbostyridiol; a 1,2,3-trihydroxynaphthalene; and dihydropyrogallol.

3. A photographic developer composition comprising an aqueous alkaline solution containing a mixture of a 3-pyrazolidone silver halide developing agent and coumarindiol.

4. A photographic developer composition comprising an aqueous alkaline solution containing a mixture of a 3-pyrazolidone silver halide developing agent and thiacoumarindiol.

5. A photographic developer composition comprising an aqueous alkaline solution containing a mixture of a 3-pyrazolidone silver halide developing agent and carbostyridiol.

6. A photographic developer composition comprising an aqueous alkaline solution containing a mixture of a 3-pyrazolidone silver halide developing agent and dihydropyrogallol.

7. A photographic developer composition comprising an aqueous alkaline solution containing a mixture of a 3-pyrazolidone silver halide developing agent and 1,2,3-trihydroxynaphthalene.

8. The developer composition of claim 1 containing 1-phenyl-3-pyrazolidone as the 3-pyrazolidone silver halide developing agent.

9. The developer composition of claim 1 containing a 1-tolyl-3-pyrazolidone as the 3-pyrazolidone silver halide developing agent.

10. The developer composition of claim 1 containing a 4,4-dialkyl-3-pyrazolidone as the 3-pyrazolidone silver halide developing agent.

11. The developer composition of claim 1 containing a 1-tolyl-4,4-dimethyl-3-pyrazolidone as the 3-pyrazolidone silver halide developing agent.

12. The developer composition of claim 1 containing 1-p-tolyl-4,4-dimethyl-3-pyrazolidone as the 3-pyrazolidone silver halide developing agent.

13. The developer composition of claim 1 containing 1-p-( $\beta$ -hydroxyethylphenyl)-3-pyrazolidone as the 3-pyrazolidone silver halide developing agent.

14. The developer composition of claim 1 containing 1-(p- $\beta$ -hydroxyethylphenyl)-4,4-dimethyl-3-pyrazolidone as the 3-pyrazolidone silver halide developing agent.

15. A photographic developer composition comprising an aqueous alkaline solution of a mixture of 1-phenyl-3-pyrazolidone and dihydropyrogallol.